

## UNITED STATES PATENT OFFICE

2,110,274

## LIGHT STABILIZER FOR HYDROCARBONS

Louis A. Mikeska, Elizabeth, and John B. Holtzclaw, Roselle, N. J., assignors to Standard Oil Development Company, a corporation of Delaware

No Drawing. Application May 25, 1935,  
Serial No. 23,452

10 Claims. (Cl. 44—9)

This invention relates to the improvement of fuels, and more particularly to the stabilization of fuels against deterioration by light, by the addition thereto of small but effective quantities of oil soluble aliphatic alcohol amine esters and the like.

Liquid fuels such as those employed in internal combustion engines, lamps, heating furnaces and the like may become "off color" or form colored 10 films or otherwise deteriorate when exposed to sunlight or other sources of actinic rays or heat, and thereby become unsuitable for their intended uses.

The object of the present invention is to overcome these difficulties by adding to the fuels, small but effective quantities of oil soluble aliphatic or aromatic alcohol amine esters, or ethers.

These esters may be obtained by the action of the corresponding acids, acid chlorides, acid anhydrides or other compounds which give esters or ethers, by reacting with aliphatic or aromatic hydroxyamines as, for example, according to the following equation:

25  $nRCOOH + (HOR')_nNH_x(RCOOR')_nNH_x + nH_2O$   
where R and R' are aliphatic or cyclic radicals, while x is any value from 0 to 2, and n is any value from 1 to 3.

The products formed according to this reaction 30 are generally recovered as the salts of the acid employed in the esterification. These salts may be neutralized with weak bases, if it be so desired, in order to produce the free amines for use according to this invention. However the salts themselves may be employed for the same purpose, and it is our intention to employ such salts or even salts containing different acid groups than those present in the ester radicals, as exemplified by the formula  $(ROOR')_nNH_xHR''$  where  $HR''$  may 35 be an aliphatic or cyclic carboxylic acid or phenol. The hydrocarbon radicals R and R' may be either normal or branched.

Although any aliphatic hydroxy compound may 40 be employed as a raw material, it is preferred to use the water-soluble amines, such as the ethanol amines, propanol amines and the like, because of their effectiveness in stabilizing fuels.

In the case of the polyhydroxy alkyl amines, it is possible to esterify sufficient hydroxy groups 45 to make the products oil-soluble, thereby often leaving some free hydroxy groups in the molecule, although it is preferable to esterify all the hydroxy groups so as to produce a more stable compound.

50 Examples of the materials suitable for the purposes of the present invention are: triacetoxy-triethanolamine ( $CH_3COOCH_2CH_2)_3N$ , triacetoxy-triethanolamine laurate, tripropionyl-triethanolamine benzoate, dibenzoyl-triethanolamine phenolate, acetylated triethanolamine salts

of hydroxystearic acid or of tertiary butyl phenol. Tributyrin, divalyryl, mono-oleyl and distearyl and similar esters of triethanolamine and similar compounds may also be used.

These compounds may be added to the fuels in 5 proportions of 0.01% to 0.5% depending on the stability of the fuel and the effectiveness of the inhibitor.

In the case of triacetoxy-triethanolamine in a freshly prepared cracked U. S. grade motor 10 gasoline, the quantity of inhibitor employed to give satisfactory results was in the neighborhood of 0.05%.

The alcoholamine esters herein described may be employed to stabilize gasolines, naphthas, 15 kerosenes and similar products with boiling ranges up to 650° F.

For instance, gasoline rich in cracked products, benzol or other cyclic materials, such as the fuels prepared by vapor phase or liquid phase cracking of petroleum oils or coal tar oils, are satisfactorily stabilized according to this invention. Blended fuels as, for example, gasoline containing alcohols, metallo-organic anti-knock compounds, dyes, lubricating agents, soaps, thickeners and the like may also be treated in the same manner.

It has now been found that triacetoxy-triethanolamine and its homologs are more effective as light stabilizers than are other amines, such as triethanolamine and butylamine which have been used for the same purpose.

Triacetoxy-triethanolamine may be made by the action of the hydroxylalkylamine with acetic acid, or the anhydride or chloride according to 35 the following equation:



## Example

40

A cracked gasoline was blended with varying quantities of triacetoxytriethanolamine and exposed to the sunlight in 4 oz. sample bottles together with a blank sample of the same gasoline. 45 The following results were obtained after the exposed sample stood for six months:

| Sample                 | Color                | Residue       | Appearance | Odor   | 50 |
|------------------------|----------------------|---------------|------------|--------|----|
| Original gasoline...   | Dark red-dish brown. | Considerable. | Cloudy...  | Rank.  |    |
| Same + 0.1% inhibitor. | Water white.         | Slight.....   | Clear..... | Sweet. |    |
| Same + 0.2% inhibitor. | Water white.         | Negligible.   | Clear..... | Sweet. | 55 |

These tests show the exceptional stabilizing properties of the inhibitors prepared according to the invention.

60

It will be understood that the invention is not limited to the description given above nor to the examples cited, and other acids and other hydroxyamines may be used to prepare other esters 5 and other compounds of the same general type as those shown in the equation which has been given.

The invention is not to be limited to any theoretical statements which have been presented 10 herein solely for purposes of illustration, but is limited only by the following claims in which it is intended to claim all novelty insofar as prior art permits.

We claim:

- 15 1. The process of stabilizing a hydrocarbon liquid which comprises adding thereto approximately 0.01 to 0.5% of a substance selected from the group consisting of esters having the general formula  $(RCOOR')_nNH_x$ , in which R is an aliphatic or aromatic hydrocarbon radical and R' is an aliphatic hydrocarbon radical while x is any value from 0 to 2 and n is any value from 1 to 3.
- 20 2. The process of stabilizing motor fuels which comprises adding thereto approximately 0.01 to 0.5% of triacetoxytriethanolamine.
- 25 3. The process of stabilizing motor fuels which comprises adding thereto approximately 0.01 to 0.5% of tripropionyltrihydroxy-trialkylamines.
- 30 4. The process of stabilizing motor fuels which comprises adding thereto approximately 0.01 to 0.5% of tributyryltriethanolamine.
- 35 5. A hydrocarbon fuel which has been stabilized against deterioration by the action of light by adding thereto approximately 0.01 to 0.5% of a substance selected from the group consisting of esters having the general formula

$(RCOOR')_nNH_x$ ,

in which R is an aliphatic or aromatic hydrocar-

bon radical and R' is an aliphatic hydrocarbon radical while x is any value from 0 to 2 and n is any value from 1 to 3.

6. A hydrocarbon fuel which has been stabilized against deterioration by the action of light by adding thereto 0.01 to 0.5% of triacetoxytriethanolamine.

7. A hydrocarbon fuel which has been stabilized against deterioration by the action of light by adding thereto 0.01 to 0.5% of tripropionyltrihydroxy-trialkylamines.

8. A hydrocarbon fuel which has been stabilized against deterioration by the action of light by adding thereto 0.01 to 0.5% of tributyryltriethanolamine.

9. The process of stabilizing a hydrocarbon liquid which comprises adding thereto from 0.01 to 0.5 percent of a substance selected from the group consisting of esters having the general formula  $(RCOOR')_nNH_x$  and in which R is an aliphatic or aromatic hydrocarbon radical and R' is an aliphatic hydrocarbon radical, while x is any value from 0 to 2 and n is any value from 1 to 3.

10. A hydrocarbon fuel which has been stabilized against deterioration by the action of light by adding thereto approximately 0.01 to 0.5% of a substance selected from the group consisting of esters having the general formula

$(RCOOR')_nNH_x$ ,

and in which R is an aliphatic or aromatic hydrocarbon radical and R' is an aliphatic hydrocarbon radical, while x is any value from 0 to 2, and n is any value from 1 to 3.

LOUIS A. MIKESKA.  
JOHN B. HOLTZCLAW.